

Patented Sept. 16, 1941

2,256,112

# UNITED STATES PATENT OFFICE

2,256,112

## YARN CONDITIONING PROCESS AND COMPOSITION THEREFOR

Joseph B. Dickey, Rochester, N. Y., assignor to  
Eastman Kodak Company, Rochester, N. Y., a  
corporation of New Jersey

No Drawing. Application September 18, 1940,  
Serial No. 357,291

15 Claims. (Cl. 28—1)

This invention relates to the treatment of cellulose organic derivative filaments, fibers, threads and the like and more particularly to a method of eliminating the tendency of such materials to accumulate charges of static electricity in twisting, winding and spinning. The invention also relates particularly to the treatment of cellulose organic derivative cut staple fibers to adapt them for the manufacture of spun yarns.

As is well-known, cellulose organic derivative materials, particularly in filament, yarn, or sheet form, are particularly subject to the accumulation on their surfaces of charges of static electricity from frictional and other influences. In the case of filaments and yarns in which the surface area of the material (per unit of weight) is enormously greater as compared to sheets or films, the problem of static often assumes serious proportions. In the manufacture of yarns of various types from artificial filaments, numerous steps in which the yarn is subjected to frictional influences may be necessary, as for example, twisting, winding, warping, carding, combing, drawing, spinning and the like, all of which operations tend to produce large accumulations of static on the filaments. This is particularly aggravated in the utilization of cut staple, as for example, in the making of spun yarn, since in carding and combing considerable friction is developed and as a result sufficient charges accumulate on the fibers to make the formation of the web difficult, if not impossible; furthermore, even if a web is formed with some degree of success, the subsequent drafting operation produces a very uneven spun yarn or intermediate roving due to the presence of the static charge. In addition, there is the ever-present fire hazard.

Cellulose derivative yarn, particularly in the form of cut staple, is extremely difficult to handle in the various operations involved in making spun yarn, not only because such material is composed of filaments having smooth, glass-like surfaces without natural kink or irregularity, but also because it has relatively negligible moisture content at normal humidities, as compared to natural fibers such as cotton and wool, making it inherently far more susceptible to the accumulation of static. The charges accumulating on cellulose derivative cut staple fibers are, under some circumstances, even sufficient to separate the individual fibers a distance of inches, notwithstanding their relatively minute size.

This invention has as its principal object to provide an improved method for the treatment of cellulose organic derivative yarns to reduce or eliminate the tendency of such yarns to accumulate charges of electricity under frictional and other influences. A further object is to provide a method of facilitating the handling and employment of cellulose organic derivative cut

staple fibers in the various operations involved in the manufacture of spun yarns. A still further object is to provide a method of treating cellulose organic derivative yarns in either filament or cut staple form, wherein the material is simultaneously softened and lubricated and the accumulation of static charges thereon is prevented. Another object is to provide an improved type of cellulose organic derivative cut staple having little or no tendency toward accumulation of static electrical charges. Other objects will appear hereinafter.

These objects are accomplished by the following invention which in its broader aspects comprises applying to cellulose organic derivative yarns either in the form of filaments, threads or staple fibers, an antistatic composition containing as its essential antistatic component a phosphonic acid of a ketone containing one or two naphthyl groups or a salt thereof. We have found that compounds having the general formula:



wherein R is a substituent selected from the group consisting of hydrogen, alkyl, alkylene, aryl, heterocyclic, cycloalkyl and naphthyl groups may be treated with hypophosphorus acid to give compounds having the formula:



wherein R has the meaning referred to above. If the reaction is stopped at the intermediate stage



mixed acids can be formed by treating with a different aldehydic or ketonic compound. These mixed acids may be represented by the formula:



wherein R has the meaning referred to above, R' and R' are similar to R and wherein R' and R' may be part of the same system of cyclic carbon atoms. Products of the type illustrated by this formula are obtained by reacting compounds of the type illustrated by the structural formula



with hypophosphorous acid and then with compounds illustrated by the structural formula



wherein R and R' have the meaning referred to above.

#### PREPARATION OF ACIDS

Intermediates required for the preparation of the new phosphonic acids of ketones of our invention are described in the copending application of J. B. Dickey and J. G. McNally Ser. No. 320,718, filed February 24, 1940, in U. S. Patents 1,988,021 and 1,989,325 and in Lewkowitsch, "Chem. Technology of Oils, Fats, and Waxes," 6th edition, 1, p. 146-155. By the term naphthyl we refer to radicals of the general class described in chapter 48 of "The Chemistry of Petroleum Derivatives" by Carleton Ellis.

Typical examples of the preparation of this type of compound are given below:

#### Example 1

3 moles of phenylnaphthyl ketone are heated with 66 g. of hypophosphorus acid for one day or more at a temperature of 60-100°. Upon cooling a product having the formula:



(bis-phenylnaphthyl hydroxy methane phosphonic acid) crystallizes out. There is also formed some



which is quickly oxidized to



#### Example 2

2.5 gram moles methylnaphthyl ketone are reacted with 66 g. of hypophosphorus acid as in Example 1. The product has the formula:



(bis-alpha-naphthyl-alpha-hydroxy ethane phosphonic acid)

#### Example 3

One-gram mole of dinaphthyl ketone is reacted with 66 g. of hypophosphorus acid as in Example 1 and the intermediate product thus formed is heated as before with two moles of methylamyl ketone. The product has the formula:



(di-naphthyl hydroxy methane-beta-hydroxy heptane phosphonic acid)

The compounds listed below represent in gen-

eral the products of this invention prepared by the technique described above.



(2-isopropyl-8-sulfo-1-naphthyl naphthyl hydroxy methane-alpha-hydroxy-alpha-cyclopentyl ethane phosphonic acid).



(bis-furyl naphthyl hydroxy methane phosphonic acid)



(bis-naphthyl hydroxy cyclohexane hydroxy methane phosphonic acid)



(bis-2-hydroxy-5-amino phenyl naphthyl hydroxy-methane phosphonic acid)



(bis-2-amino-5-dimethyl amino phenyl naphthyl hydroxy-methane phosphonic acid)

#### PREPARATION OF SALTS

One mole of



is treated in water with 1 mole potassium hydroxide. The product, potassium bis-naphthyl acetoxy stearyl methane phosphonic acid salt, is slightly soluble in hot water. In place of potassium I may prepare the sodium, am-

monium, calcium, barium, magnesium, etc., salts.

*Example 5*

One mole of



is reacted with triethanolamine in the dry state or in any suitable solvent. The salt formed is bis - alpha - naphthyl - alpha - hydroxy - ethane phosphonic acid triethanolamine salt. In place of triethanolamine I may use ethanolamine, diethanolamine, glycerolamine, mono-, di-, or tri-butylamine, cyclohexylamine, diethylcyclohexylamine, tetrahydrofurfurylamine, ditetrahydrofurfurylamine, di-beta-alkoxy-ethyl-amine, morpholine, ethylenediamine, tetramethylammonium hydroxide, etc.

In accordance with my invention, the above-mentioned compounds may be applied to the yarn in any convenient manner, for example, by roll, wick, immersion, spraying or the like. Inasmuch as these compounds are soluble in oil they may be dissolved or dispersed in oils such as mineral oil, blown and unblown, drying, and semi-drying, vegetable and animal oils, examples of which are light mineral, neat's-foot, olive, tea-seed, castor, soya bean, rapeseed oils, etc., and other lubricants.

In the following examples and description, I have set forth several of the preferred embodiments of my invention, but they are included merely for purposes of illustration and not as a limitation thereof.

*Example 6*



is applied to textile materials (silk, wool, viscose, cotton, cellulose acetate) by means of a wick, bath, roller, spray, etc., to facilitate their knitting, weaving, spinning, and the like. Yarns lubricated with the above types of lubricants are of special value in the preparation of cut staple fibers. These fibers may be oiled before or after cutting.

*Example 7*

A conditioning liquid is made up as follows:



and applied to textile materials such as silk, wool, cotton, viscose, cellulose acetate, etc., as described in Example 6. If the yarn is intended primarily for knitting, the amount of conditioning liquid applied may vary from 2-25% by weight of the yarn and if for weaving, between 1-5% by weight.

Cellulose acetate filaments treated as described

above are quite soft and pliable and give improved results in textile operations such as weaving, knitting, etc., and especially in the preparation of cut staple yarn. Other examples of suitable lubricating mixtures having antistatic properties which are used as illustrated in Examples 6 and 7 follow.

*Example 8*



## Example 15

|                                                                                        |          |
|----------------------------------------------------------------------------------------|----------|
| Blown sperm oil.....                                                                   | Parts 68 |
|       | 10       |
| (bis-naphthyl phenyl hydroxy methane phosphonic acid tri-beta-methoxyethyl amine salt) | 5        |
| Water.....                                                                             | 20       |

Di-beta-methoxyethyl succinate.....

## Example 16

|                                                                                   |            |
|-----------------------------------------------------------------------------------|------------|
|  | Parts 1-10 |
| (bis-alpha-tetralin-1-dimethylamino-2-alpha-hydroethane phosphonic acid)          | 20         |

Teased oil.....

|                                                                                    |             |
|------------------------------------------------------------------------------------|-------------|
| Blown teased oil.....                                                              | Parts 38-20 |
| Glycerolacetone acetate.....                                                       | 50-70       |
|   | 1-5         |
| (bis-alpha-naphthyl-beta-methoxy ethane phosphonic acid benzylamine salt)          | 30          |
|  | 1-5         |
| (Beta-hydroxy propane phosphonic acid diethyliclohexyl amine salt)                 | 35          |

## Example 18

|                                                                                            |            |
|--------------------------------------------------------------------------------------------|------------|
|         | Parts 1-10 |
| (bis-naphthyl oleyl (sulfonated) hydroxy methane phosphonic acid bis cyclohexylamine salt) | 45         |

Blown olive oil.....

Blown neat's foot oil.....

## Example 19

|                        |             |
|------------------------|-------------|
| Olive oil.....         | Parts 55-60 |
| Sulfonated castor..... | 10          |
| Mineral oil.....       | 20          |
| Oleic acid.....        | 10-15       |



## Example 20

|                                                                                     |          |
|-------------------------------------------------------------------------------------|----------|
| Water.....                                                                          | Parts 65 |
| Water soluble cellulose ester.....                                                  | 70       |
|  | 15       |
| (methyl naphthyl hydroxy methane-alpha-hydroxy ethane phosphonic acid sodium salt)  | 5        |
| Sulfonated olive oil.....                                                           | 70       |

## Example 21

One pound of 1 - methylamino - 4-ethylamino-anthraquinone is ground with  $\frac{1}{4}$  pound of



and three pounds of sugar. The resulting finely divided mixture is then added to 100 gallons water heated to 60-80° and the resulting aqueous suspension is used to dye about 100 pounds cellulose acetate.

Any of the above compositions may be applied to the yarn intended for use in circular knitting by means of a bath, wick, spray, roller, pad or any suitable means. The amount of conditioning liquid applied may vary between 5-25% by weight of the yarn. Usually, however, the amount of conditioning liquid applied is about 10-15% by weight of the yarn. Yarn composed of cellulose acetate conditioned as described above gives excellent results when used in the circular knitting process.

If the conditioning agent is to be applied to the yarn after spinning, this may be done by bringing the yarn in contact with a wick, roll, or felt wet therewith, or the liquid may be applied by immersion, spray, or otherwise. The particular point at which the liquid is applied may vary. It may, for example, be applied to the yarn inside or outside the spinning cabinet, between the guide and godet roll, between the godet or other roll or guide and the point of winding and/or twisting. In some cases, the liquid may even be applied to the yarn after winding onto cones, spools, bobbins, or the like or by the so-called "bobbin to bobbin" method. In the case of staple fiber manufacture, the liquid may be applied to the yarn prior to, or after cutting into staple lengths.

The amount of the agent so employed will vary widely depending upon the results desired, the specific nature of the material to which the agent is applied, the use to which the yarn is eventually to be put and other factors. For example, in a given case where a cellulose organic acid ester is intended for knitting, about 4 to 25% or more by weight, based on the weight of the dry yarn, may be satisfactory, while if the yarn is intended for weaving, the amount may vary between about 1 and 5%.

Although in the above examples I have referred primarily to yarn treating compositions containing only the conditioning agent and an oil, other ingredients such as solvents, non-solvents, emulsifying agents, blending agents and the like, may be added within the scope of my invention. Likewise, various dyes or other coloring matter may be included in case it is desired to permanently or fugitively tint or dye the material undergoing treatment.

Although I have found it convenient to illustrate my invention by reference to compositions containing specific percentages of the various ingredients, these percentages may vary widely depending upon the particular purpose for which the composition is intended. For example, if it is desired to control the deelectrifying action of the conditioning agent, the amount of the agent may be adjusted as, for example, by reducing the amount of the agent and correspondingly increasing the amount of oil or other ingredient. While I have described my invention with par-

ticular reference to the treatment of yarns composed of organic derivatives of cellulose such as cellulose acetate, the conditioning agents and formulas described herein are applicable to the conditioning of many other types of cellulose derivative yarns such as those composed of or containing cellulose propionate, cellulose butyrate, cellulose acetate propionate, cellulose acetate butyrate, ethyl cellulose, methyl cellulose, benzyl cellulose and others, as well as to the conditioning of silk, wool, cotton, viscose and other natural or artificial materials.

The term "yarn" as used herein and in the claims is to be understood as including a single filament, a plurality of filaments associated into the form of a thread, either of high or low twist, single or multiple threads associated or twisted together, composite threads composed of a mixture of natural and artificial filaments or a composite thread formed by twisting together individual strands of natural or artificial materials, as well as cut staple fibers produced from natural and/or artificial filaments or threads and spun yarn produced from such staple fibers.

As indicated above, the yarn conditioning agents of my invention are exceptionally good solvents for a wide variety of mineral, blown and unblown, drying and semi-drying animal and vegetable oils such as cottonseed, olive, castor, neat's-foot, sperm and other oils. This enables them to be used with any of such oils in making up a variety of yarn treating formulas of varying composition.

The yarn conditioning agents of my invention also have exceptional value as surface-active compounds and as such may be employed as wetting agents, emulsifying and dispersing agents, textile assistants, dye dispersing agents and the like.

The yarn conditioning method and compositions of my invention possess many outstanding advantages. The fundamental and outstanding characteristic of the agents employed in accordance with the invention is their ability to de-electrify yarns, especially those composed of or containing organic derivatives of cellulose such as cellulose acetate and render them amenable to various textile operations, especially operations such as those involved in the manufacture of cut staple fibers, as well as in weaving and knitting. Another outstanding characteristic of these compounds is their exceptional solvent power for a wide variety of mineral, animal, and vegetable oils and their ability to act as lubricating assistants in conjunction with these oils when applied to such yarns.

In addition, due to their solubility in water, they may be readily removed from yarns and fabrics by means of the usual aqueous scour baths.

Of the above compositions I have found that bisphenyl naphthyl hydroxy methane phosphonic acid, bis-alpha-naphthyl-alpha-hydroxy ethane phosphonic acid, and bis-naphthyl hydroxy methane phosphonic acid are outstanding in their ability to reduce or eliminate the tendency of yarns composed of or containing organic derivatives of cellulose to accumulate charges of static electricity.

What I claim is:

1. The method of eliminating the tendency of yarns, filaments or fibers to accumulate charges of static electricity, which comprises applying thereto a composition containing as its

essential anti-static component a phosphonic acid of a ketone having the general formula:



wherein R is a substituent selected from the group consisting of hydrogen, alkyl, alkylene, aryl, heterocyclic, cycloalkyl and naphthyl.

2. The method of eliminating the tendency of yarns, filaments or fibers composed of or containing organic derivatives of cellulose to accumulate charges of static electricity, which comprises applying thereto a composition containing as its essential anti-static component a phosphonic acid of a ketone having the general formula:



wherein R is a substituent selected from the group consisting of hydrogen, alkyl, alkylene, aryl, heterocyclic, cycloalkyl and naphthyl.

3. The method of eliminating the tendency of yarns, filaments or fibers composed of or containing cellulose acetate to accumulate charges of static electricity, which comprises applying thereto a composition containing as its essential anti-static component a phosphonic acid of a ketone having the general formula:



40 wherein R is a substituent selected from the group consisting of hydrogen, alkyl, alkylene, aryl, heterocyclic, cycloalkyl and naphthyl.

4. The method of eliminating the tendency of yarns, filaments or fibers composed of or containing organic derivatives of cellulose to accumulate charges of static electricity, which comprises applying thereto a composition containing as its essential anti-static component bis-phenyl-naphthyl hydroxy methane phosphonic acid.

5. The method of eliminating the tendency of yarns, filaments or fibers composed of or containing organic derivatives of cellulose to accumulate charges of static electricity, which comprises applying thereto a composition containing as its essential anti-static component bis-alpha-naphthyl-alpha-hydroxy ethane phosphonic acid.

6. The method of eliminating the tendency of yarns, filaments or fibers composed of or containing organic derivatives of cellulose to accumulate charges of static electricity, which comprises applying thereto a composition containing as its essential anti-static component bis-naphthyl hydroxy methane phosphonic acid.

65 7. Textile yarns having a lessened tendency to accumulate charges of static electricity, said yarns containing a phosphonic acid of a ketone having the general formula:



70 75 wherein R is a substituent selected from the

group consisting of hydrogen, alkyl, alkylene, aryl, heterocyclic, cycloalkyl and naphtharyl.

8. Textile yarns composed of or containing organic derivatives of cellulose having a lessened tendency to accumulate charges of static electricity, said yarns containing a phosphonic acid of a ketone having the general formula:



wherein R is a substituent selected from the group consisting of hydrogen, alkyl, alkylene, aryl, heterocyclic, cycloalkyl and naphtharyl.

9. Textile yarns composed of or containing cellulose acetate having a lessened tendency to accumulate charges of static electricity, said yarns containing a phosphonic acid of a ketone having the general formula:



wherein R is a substituent selected from the group consisting of hydrogen, alkyl, alkylene, aryl, heterocyclic, cycloalkyl and naphtharyl.

10. Textile yarns composed of or containing cellulose acetate having a lessened tendency to accumulate charges of static electricity, said yarns containing a phosphonic acid of a ketone having the general formula:



wherein R is a substituent selected from the group consisting of hydrogen, alkyl, alkylene,

aryl, heterocyclic, cycloalkyl and naphtharyl, and a textile lubricant.

11. Textile yarns composed of or containing organic derivatives of cellulose having a lessened tendency to accumulate charges of static electricity, said yarns containing bis-phenylnaphthyl hydroxy methane phosphonic acid.

12. Textile yarns composed of or containing organic derivatives of cellulose having a lessened tendency to accumulate charges of static electricity, said yarns containing bis-alpha-naphthyl-alpha-hydroxy ethane phosphonic acid.

13. Textile yarns composed of or containing organic derivatives of cellulose having a lessened tendency to accumulate charges of static electricity, said yarns containing bis-naphthyl hydroxy methane phosphonic acid.

14. A textile yarn anti-static composition containing as its essential anti-static component a phosphonic acid having the general formula:



wherein R is a substituent selected from the group consisting of hydrogen, alkyl, alkylene, aryl, heterocyclic, cycloalkyl and naphtharyl.

15. A textile yarn anti-static composition containing as its essential anti-static component a phosphonic acid having the formula:



where R, R<sup>1</sup> and R<sup>2</sup> are substituents selected from the group consisting of hydrogen, alkyl, alkylene, aryl, heterocyclic, cycloalkyl and naphtharyl groups and wherein R<sup>1</sup> and R<sup>2</sup> may be part of the same system of cyclic carbon atoms.

JOSEPH B. DICKEY.